



US011110468B2

(12) **United States Patent**  
**Gilbert et al.**

(10) **Patent No.:** **US 11,110,468 B2**  
(45) **Date of Patent:** **Sep. 7, 2021**

(54) **SEPARATION OF A MIXTURE USING MAGNETIC CARRIER PARTICLES**

- (71) Applicant: **BASF SE**, Ludwigshafen am Rhein (DE)
- (72) Inventors: **David Johann Gilbert**, Villach (AT); **Wolfgang Rohde**, Ludwigshafen am Rhein (DE); **Michael Mentges**, Ludwigshafen am Rhein (DE); **Rodrigo Enrique Munizaga**, Santiago (CL); **Oliver Kuhn**, Ludwigshafen am Rhein (DE); **Bernhard Schuler**, Ludwigshafen am Rhein (DE)
- (73) Assignee: **BASF SE**, Ludwigshafen am Rhein (DE)

(\*) Notice: Subject to any disclaimer, the term of this patent is extended or adjusted under 35 U.S.C. 154(b) by 0 days.

(21) Appl. No.: **16/627,846**

(22) PCT Filed: **Aug. 2, 2018**

(86) PCT No.: **PCT/EP2018/070967**

§ 371 (c)(1),  
(2) Date: **Dec. 31, 2019**

(87) PCT Pub. No.: **WO2019/025524**

PCT Pub. Date: **Feb. 7, 2019**

(65) **Prior Publication Data**

US 2020/0122160 A1 Apr. 23, 2020

(30) **Foreign Application Priority Data**

Aug. 3, 2017 (EP) ..... 17184800  
Sep. 12, 2017 (EP) ..... 17190688

(51) **Int. Cl.**

**B03C 1/01** (2006.01)  
**H01F 1/03** (2006.01)  
**B03C 1/32** (2006.01)

(52) **U.S. Cl.**

CPC ..... **B03C 1/01** (2013.01); **B03C 1/32** (2013.01); **H01F 1/0315** (2013.01); **B03C 2201/18** (2013.01)

(58) **Field of Classification Search**

CPC ..... B03C 1/01; B03C 2201/18  
See application file for complete search history.

(56) **References Cited**

U.S. PATENT DOCUMENTS

- 4,657,666 A 4/1987 Snook et al.  
4,834,898 A 5/1989 Hwang  
5,051,199 A 9/1991 Barwise  
2012/0000857 A1\* 1/2012 Domke ..... B03C 1/015  
210/695  
2012/0228413 A1 9/2012 Rieger et al.  
2016/0317951 A1\* 11/2016 Incera Garrido ..... B03C 1/01  
2017/0274389 A1\* 9/2017 Shishkov ..... B03C 1/01

FOREIGN PATENT DOCUMENTS

|    |               |      |                        |
|----|---------------|------|------------------------|
| CL | 2008002609    | A1   | 10/2009                |
| CL | 2011002075    | A1   | 12/2011                |
| CL | 2016001761    | A1   | 12/2016                |
| CL | 2017001308    | A1   | 2/2018                 |
| EP | 1200408       | A2   | 5/2002                 |
| WO | 02/66168      | A1   | 8/2002                 |
| WO | 2007/008322   | A1   | 1/2007                 |
| WO | 2010/097361   | A1   | 9/2010                 |
| WO | 2012/028701   | A2   | 3/2012                 |
| WO | 2012/140065   | A1   | 10/2012                |
| WO | 2014/068142   | A1   | 5/2014                 |
| WO | 2015/110555   | A1   | 7/2015                 |
| WO | WO-2015104324 | A1 * | 7/2015 ..... B03C 1/01 |
| WO | WO-2016083491 | A1 * | 6/2016 ..... B03C 1/01 |

OTHER PUBLICATIONS

International Preliminary Report on Patentability received for PCT Patent Application No. PCT/EP2018/070967, dated Feb. 13, 2020, 10 pages.

International Search Report and Written Opinion received for PCT Patent Application No. PCT/EP2018/070967, dated Oct. 26, 2018, 11 pages.

Gray et al., Extractive Metallurgy Conference, Perth, Oct. 2-4, 1991, pp. 223-226.

Rushton et al., Power Characteristics of mixing impellers Part I, Chem. Eng. Progr., 46(8):395-404 (1950).

Rushton et al., Power Characteristics of mixing impellers Part II, Chem. Eng. Progr., 46(9):467-476 (1950).

Vusse, Mixing by agitation of miscible liquids Part I, Chem. Eng. Sci., 4(4):178-200 (1955).

Vusse, Mixing by agitation of miscible liquids Part II, Chem. Eng. Sci., 4(5):209-220 (1955).

\* cited by examiner

*Primary Examiner* — Bradley R Spies

(74) *Attorney, Agent, or Firm* — Faegre Drinker Biddle & Reath LLP

(57) **ABSTRACT**

The present invention relates to a process for separating at least one first material from a mixture comprising this at least one first material, at least one second material and at least one third material, which comprises at least the following steps: (A) providing a mixture comprising at least one first material, at least one second material, at least one third material and at least one hydrocarbon in an amount of more than 0.4% by weight, based on the sum of mixture, in the presence or 10 absence of at least one dispersion medium, (B) if appropriate, addition of at least one dispersion medium to the mixture obtained in step (A) in order to obtain a dispersion, (C) treatment of the dispersion from step (A) or (B) with at least one hydrophobic magnetic particle, so that the at least one first material and the at least one magnetic particle agglomerate, (D) separation of the adduct from step (C) from the mixture by application of a magnetic field, (E) if appropriate, dissociation of the adduct which has been separated off in step (D) in order to obtain the at least one first material and the at least one magnetic particle separately.

**12 Claims, No Drawings**

## 1

SEPARATION OF A MIXTURE USING  
MAGNETIC CARRIER PARTICLESCROSS-REFERENCE TO RELATED  
APPLICATIONS

This application is a national stage application (under 35 U.S.C. § 371) of PCT/EP2018/070967, filed Aug. 2, 2018, which claims benefit of European Application Nos. 17184800.5, filed Aug. 3, 2017, and 17190688.6, filed Sep. 12, 2017, all of which are incorporated herein by reference in their entirety.

The present invention relates to a process for separating at least one first material from a mixture comprising this at least one first material, at least one second material and at least one third material, wherein a mixture comprising this at least one first material, at least one second material, at least one third material and at least one hydrocarbon in an amount of more than 0.4% by weight, based on the sum of mixture, is further brought into contact with at least one hydrophobic magnetic particle so that the magnetic particle and the at least one first material agglomerate and this agglomerate is separated from the at least one second material and the at least one third material by application of a magnetic field and, if appropriate, the at least one first material is subsequently separated, preferably quantitatively, from the magnetic particle, with the magnetic particle preferably being able to be recirculated to the process.

In particular, the present invention relates to a process for separating at least one ore from a mixture in the presence of at least one further ore and the gangue. Processes for separating ores from mixtures comprising these are already known from the prior art.

WO 02/0066168 A1 relates to a process for separating ores from mixtures comprising these, in which suspensions or slurries of these mixtures are treated with particles which are magnetic and/or able to float in aqueous solutions. After addition of the magnetic and/or floatable particles, a magnetic field is applied so that the agglomerates are separated off from the mixture. However, the degree of binding of the magnetic particles to the ores and the strength of the bond is not sufficient to carry out the process with sufficiently high yield and effectiveness.

U.S. Pat. No. 4,657,666 discloses a process for the enrichment of ores, wherein the ore present in the gangue is reacted with magnetic particles, as a result of which agglomerates are formed due to hydrophobic interactions. The magnetic particles are hydrophobized on the surface by treatment with hydrophobic compounds, so that binding to the ore occurs. The agglomerates are then separated from the mixture by means of a magnetic field. Said document also discloses that the ores are treated with a surface-activating solution of 1% of sodium ethylxanthogenate before the magnetic particle is added. Ore and magnetic particle are separated in this process by destruction of the surface-activating substance which has been applied in the form of the surface-activating solution to the ore.

U.S. Pat. No. 4,834,898 discloses a process for separating off nonmagnetic materials by bringing them into contact with magnetic reagents which are enveloped by two layers of surface-active substances. U.S. Pat. No. 4,834,898 further discloses that the surface charge of the nonmagnetic particles which are to be separated off can be influenced by various types and concentrations of electrolyte reagents. For example, the surface charge is altered by addition of multivalent anions, for example tripolyphosphate ions.

## 2

S. R. Gray, D. Landberg, N. B. Gray, Extractive Metallurgy Conference, Perth, 2-4 Oct. 1991, pages 223-226 discloses a process for recovering small gold particles by bringing the particles into contact with magnetite. Before contacting, the gold particles are treated with potassium amylixanthogenate. A process for separating the gold particles from at least one hydrophilic material is not disclosed in this document.

WO 2007/008322 A1 discloses a magnetic particle which 10 is hydrophobized on the surface for the separation of impurities from mineral substances by magnetic separation processes. According to WO 2007/008322 A1, a dispersant selected from among sodium silicate, sodium polyacrylate or sodium hexametaphosphate can be added to the solution 15 or dispersion.

WO 2010/097361 A1 discloses a process for separating at least one first material from a mixture comprising this at least one first material, at least one second material and at least one third material, wherein the mixture to be treated is 20 firstly brought into contact with at least one hydrocarbon in an amount of from 0.01 to 0.4% by weight, based on the sum of mixture and at least one hydrocarbon, this mixture is further brought into contact with at least one hydrophobic magnetic particle so that the magnetic particle and the at least one first material agglomerate and this agglomerate is separated from the at least one second material and the at least one third material by application of a magnetic field and, if appropriate, the at least one first material is subsequently separated, preferably quantitatively, from the magnetic particle, with the magnetic particle preferably being 25 able to be re-circulated to the process.

It is an object of the present invention to provide a process by means of which at least one first material can be separated 30 efficiently from mixtures comprising at least one first material, at least one second material and at least one third material, where the at least one first material and the at least one second material have an identical or similar character. For example, the at least one first material and the at least one second material can be ionic compounds having the 35 same anion but different cations, for example two sulfides of different transition metal cations. Furthermore, it is an object of the present invention to treat the at least one first material to be separated off in such a way that the adduct of magnetic particle and first material is sufficiently stable to ensure a 40 high yield of the first material in the separation without a large amount of second material being separated off at the same time.

These objects are achieved by a process for separating at least one first material from a mixture comprising this at least one first material, at least one second material and at least one third material, which comprises at least the following steps:

- (A) providing a mixture comprising at least one first material, at least one second material, at least one third material and at least one hydrocarbon in an amount of more than 0.4% by weight, based on the sum of mixture, in the presence or absence of at least one dispersion medium,
- (B) if appropriate, addition of at least one dispersion medium to the mixture obtained in step (A) in order to obtain a dispersion,
- (C) treatment of the dispersion from step (A) or (B) with at least one hydrophobic magnetic particle, so that the at least one first material and the at least one magnetic particle agglomerate,
- (D) separation of the adduct from step (C) from the mixture by application of a magnetic field,

(E) if appropriate, dissociation of the adduct which has been separated off in step (D) in order to obtain the at least one first material and the at least one magnetic particle separately.

The process of the invention is preferably employed for separating at least one first, hydrophobic or hydrophobized material from a mixture comprising this at least one first, hydrophobic or hydrophobized material, at least one second, hydrophobic or hydrophobized material and at least one third, hydrophilic material, where the at least one first material and the at least one second material have a different hydrophobicity or are hydrophobized to different extents.

For the purposes of the present invention, materials are referred to as "hydrophobic" when their surface forms a contact angle against water of more than 90°. The larger the contact angle formed, the more hydrophobic the material. For the purposes of the present invention, materials are referred to as "hydrophilic" when their surface forms a contact angle against water of less than 90°. The smaller the contact angle formed, the more hydrophilic the material. In a preferred embodiment, the at least one first material has a greater hydrophobicity than the at least one second material. According to the invention, the at least one first material and, if appropriate, the at least one second material can, if appropriate, be hydrophobized by addition of a hydrophobizing agent in order to have a hydrophobicity suitable for the process of the invention.

In a preferred embodiment of the process of the invention, the at least one first material and the at least one second material are hydrophobic or hydrophobized metal compounds and the at least one third material is a hydrophilic metal compound.

Thus, the at least one first material to be separated off and the at least one second material are preferably metal compounds selected from the group consisting of sulfidic ores, oxidic and/or carbonate-containing ores, for example azurite  $[Cu_3(CO_3)_2(OH)_2]$  or malachite  $[Cu_2[(OH)_2|CO_3]]$ , and the noble metals, where the at least one first material is preferably more hydrophobic than the at least one second material. In another embodiment, the at least one second material is identical to the at least one first material.

The at least one third material which is present in the mixture to be treated according to the invention is preferably a hydrophilic metal compound selected from the group consisting of oxidic and hydroxidic metal compounds, for example silicon dioxide  $SiO_2$ , silicates, aluminosilicates, for example feldspars, for example albite  $Na(Si_3Al)O_8$ , mica, for example muscovite  $KAl_2[(OH,F)_2AlSi_3O_10]$ , garnets  $(Mg, Ca, Fe^{II})_3(Al, Fe^{III})_2(SiO_4)_3, Al_2O_3, FeO(OH), FeCO_3, Fe_2O_3, Fe_3O_4$  and further related minerals and mixtures thereof.

Examples of sulfidic ores which can be used according to the invention are, for example, selected from the group of copper ores consisting of covellite  $CuS$ , molybdenite (molybdenum(IV) sulphide), chalcopyrite (copper pyrite)  $CuFeS_2$ , bornite  $Cu_5FeS_4$ , chalcocite (copper glance)  $Cu_2S$ , pentlandite (Ni,Fe)S, pyrrhotite  $Fe_{1-x}S$ , pyrite  $FeS_2$  and mixtures thereof.

Accordingly, preference is given to using untreated ore mixtures which can be obtained from mines in the process of the invention. In another embodiment preference is given to using ore mixtures which can be obtained from mines in the process of the invention.

Very particularly preferred first materials are selected from the group consisting of molybdenum(IV) sulfide, pyrrhotite  $Fe_{1-x}S$ , chalcopyrite (copper pyrite)  $CuFeS_2$ , bornite  $Cu_5FeS_4$  and mixtures thereof. Further examples of the at

least one first material which is separated off by means of the process of the invention are noble metals, for example Au, Pt, Pd, Rh, etc., preferably in the native state or as sulfides or embedded in other minerals e.g. pentlandite (Ni,Fe)S.

Very particularly preferred second materials are selected from the group consisting of copper sulfides, for example chalcopyrite (copper pyrite)  $CuFeS_2$ , covellite  $CuS$ ,  $Cu_2S$ , pyrite  $FeS_2$  and mixtures thereof.

Depending on the conditions set (pH, redox potential of 10 the suspension, etc.),  $CuS$ ,  $Cu_2S$ ,  $ZnS$ ,  $PbS$ , bornite  $Cu_5FeS_4$  can be counted as either first materials or second materials. This is known to those skilled in the art.

The present invention also provides a process according to the invention in which the at least one first material is a sulfidic molybdenum ore and the at least one second material is a sulfidic copper ore.

The present invention further provides a process according to the invention in which the at least one first material is chalcopyrite (copper pyrite)  $CuFeS_2$  and the at least one second material is  $ZnS$ .

The present invention further provides a process according to the invention in which the at least one first material is  $Cu_2S$  and the at least one second material is pyrite  $FeS_2$ .

The present invention also provides a process according to the invention in which the at least one third material is selected from the group consisting of oxidic and hydroxidic metal compounds.

Very particularly preferred third materials are selected from among silicon dioxide  $SiO_2$ , feldspar  $(Ba, Ca, Na, K, NH_4)(Al, B, Si)_4O_8$ , limestone  $CaCO_3$ , dolomite  $(Ca, Mg)CO_3$ , mica  $KAl_2[AlSi_3O_10(OH)_2]$ , olivine  $(Mg, Mn, Fe)_2[SiO_4]$ , clay minerals and mixtures thereof.

In addition to the compounds mentioned, sulfides of metals other than copper, for example sulfides of iron, lead, 35 zinc or molybdenum, i.e.  $FeS/FeS_2$ ,  $PbS$ ,  $ZnS$ , can also be present in the mixtures. Furthermore, oxidic compounds of metals and semimetals, for example silicates or borates, or other salts of metals and semimetals, for example phosphates, sulfates or oxides/hydroxides/carbonates and further salts, for example azurite  $[Cu_3(CO_3)_2(OH)_2]$ , malachite  $[Cu_2[(OH)_2|CO_3]]$ , barite  $(BaSO_4)$ , monazite  $((La-Lu)PO_4)$  can be present in the ore mixtures to be treated according to the invention.

Thus, a particularly preferred mixture which is treated in the process of the invention comprises molybdenum(IV) sulfide, chalcopyrite (copper pyrite)  $CuFeS_2$  or  $Cu_2S$  as first material, copper sulfide, for example  $CuS$  and/or  $Cu_2S$ ,  $ZnS$  or pyrite  $FeS_2$  as second material and silicon dioxide  $SiO_2$  and possibly further oxides and/or hydroxides as third material.

In the mixture to be provided in step (A), the at least one first material is preferably present in an amount of from 0.001 to 5.0% by weight, more preferably from 0.01 to 1% by weight, particularly preferably from 0.01 to 0.1% by weight, in each case calculated as metal and based on the total amount of the at least one first material, the at least one second material and the at least one third material. In another embodiment, in the mixture to be provided in step (A), the at least one first material is preferably present in an amount of from 0.0001 to 50% by weight, more preferably from 0.001 to 40% by weight, particularly preferably from 0.01 to 0.20% by weight, in each case calculated as metal and based on the total amount of the at least one first material, the at least one second material and the at least one third material.

In the mixture to be provided in step (A), the at least one second material is preferably present in an amount of from 0.1 to 5.0% by weight, more preferably from 0.5 to 4.0% by

weight, in each case calculated as metal and based on the total amount of the at least one first material, the at least one second material and the at least one third material.

In the mixture to be provided in step (A), the at least one third material is generally present in such an amount that the sum of the at least one first material, the at least one second material and the at least one third material is 100% by weight.

Further to the at least one first material, the at least one second material and the at least one third material, at least one hydrocarbon is present in the mixture to be provided in step (A). The amount of the at least one hydrocarbon is more than 0.4% by weight based on the total amount of the at least one first material, the at least one second material, the at least one third material and the at least one hydrocarbon.

In a preferred embodiment of the process of the invention, the mixture comprising at least one first material, at least one second material and at least one third material is present in step (A) in the form of particles having a size of from 100 nm to 500  $\mu\text{m}$ , for example <125  $\mu\text{m}$ , see, for example, U.S. Pat. No. 5,051,199. In a preferred embodiment, this particle size is obtained by milling. Suitable processes and apparatuses are known to those skilled in the art, for example wet milling in a ball mill.

In a preferred embodiment of the process of the invention, the mixture comprising at least one first material and at least one second material is therefore milled to particles having a size of from 100 nm to 500  $\mu\text{m}$ , preferably from 100 nm to 100  $\mu\text{m}$ , for example <125  $\mu\text{m}$ , before or during step (A).

An ore mixture which is typically used for separation by means of the process of the invention has the following composition: about 30% by weight of  $\text{SiO}_2$ , about 30% by weight of feldspar, about 2% of  $\text{FeCuS}_2$ , about 0.5% of  $\text{Cu}_5\text{FeS}_4$ , about 0.04% by weight of  $\text{MoS}_2$ , balance chromium, iron, titanium, manganese and magnesium oxides. Another ore mixture which is typically used for separation by means of the process of the invention has the following composition: about 1% by weight of  $\text{SiO}_2$ , about 1% by weight of feldspar, about 3% of  $\text{FeCuS}_2$ , 10% pyrophyllite, 10% Kaolinite about 70% by weight of  $\text{MoS}_2$ , balance chromium, iron, titanium, manganese, aluminium, silicon and magnesium oxide minerals.

The individual steps of the process of the invention are described in detail below:

#### Step (A):

Step (A) of the process of the invention comprises providing a mixture comprising at least one first material, at least one second material, at least one third material and at least one hydrocarbon in an amount of more than 0.4% by weight, based on the sum of mixture, in the presence or absence of at least one dispersion medium.

Suitable and preferred first, second and third materials have been mentioned above.

For the purposes of the present invention, a hydrocarbon is an organic chemical compound which is made up essentially of carbon, hydrogen and possibly oxygen. If oxygen is present in addition to carbon and hydrogen in the hydrocarbons which can be used according to the invention, it is present, for example, in the form of ester, carboxyl and/or ether groups. Either an essentially uniform hydrocarbon or a hydrocarbon mixture can be used in step (A) of the process of the invention.

Hydrocarbons or hydrocarbon mixtures which can be used according to the invention generally have a low viscosity under the conditions of the process of the invention, so that they are liquid and mobile under the process conditions according to the invention. Preference is given to using

hydrocarbons or hydrocarbon mixtures which have a viscosity of from 0.1 to 100 cP, preferably from 0.5 to 5 cP, in each case at 20° C.

Hydrocarbons or hydrocarbon mixtures which can be used according to the invention generally have a flash point of  $\geq 20^\circ \text{C}$ ., preferably  $\geq 40^\circ \text{C}$ . The present invention therefore also provides the process according to the invention in which the at least one hydrocarbon has a flash point of  $\geq 20^\circ \text{C}$ ., particularly preferably  $\geq 40^\circ \text{C}$ .

In a preferred embodiment of the process of the invention, the at least one hydrocarbon is selected from the group consisting of mineral oils, vegetable oils, biodiesel, BtL (Biomass-to-Liquid) fuels, products of coal liquefaction, products of the GtL (Gas to Liquid, from natural gas) process and mixtures thereof.

Mineral oils are, for example, crude oil derivatives and/or oils produced from brown coal, hard coal, peat, wood, petroleum and, if appropriate, other mineral raw materials by distillation. Mineral oils generally comprise hydrocarbon mixtures of paraffinic hydrocarbons, i.e. saturated chain-like hydrocarbons, naphthenic hydrocarbons, i.e. saturated cyclic hydrocarbons, and aromatic hydrocarbons.

A particularly preferred crude oil derivative is diesel or gas oil. Diesel generally has a composition known to those skilled in the art. Diesel is based essentially on mineral oil, i.e. diesel is a fraction in the fractionation of mineral oil by distillation. The main constituents of diesel are predominantly alkanes, cycloalkanes and aromatic hydrocarbons having from about 9 to 22 carbon atoms per molecule and a boiling range from 170° C. to 390° C.

Further names for suitable petroleum derivatives comprise: light gas oil (boiling point 235-300° C., also referred to, depending on the specification, as "diesel", "diesel fuel", "DF", "light heating oil", "LHO"), heavy gas oil (boiling point 300-375° C.) and also (in the USA) "No. 2 fuel".

Vegetable oils are generally fats and fatty oils which are obtained from oil plants. Vegetable oils comprise, for example, triglycerides. Vegetable oils which are suitable for the purposes of the invention are, for example, selected from the group consisting of sunflower oil, rapeseed oil, safflower oil, soybean oil, corn oil, peanut oil, olive oil, herring oil, cotton seed oil, palm oil and mixtures thereof.

Biodiesel generally has a composition known to those skilled in the art. Biodiesel comprises essentially methyl esters of saturated  $\text{C}_{16}$ - $\text{C}_{18}$ -fatty acids and unsaturated  $\text{C}_{18}$ -fatty acids, in particular the methyl ester of rapeseed oil.

Products of coal liquefaction can, for example, be obtained by the Fischer-Tropsch or Sasol process. The BtL and GtL processes are known to those skilled in the art.

In a preferred embodiment of the process of the invention, diesel, kerosene and/or light gas oil is used as hydrocarbon in step (A). On a laboratory scale, diesel of the brands Solvesso® and/or Shellsol® can advantageously be used.

In step (A) of the process of the invention, at least one hydrophobizing agent may, if appropriate, be additionally added. For the purposes of the present invention, a "hydrophobizing agent" is a substance which is able to increase the hydrophobicity of the surface of the at least one first material in the presence of the other particles which are not to be separated off. Hydrophobizing agents which can be used according to the invention become attached to the at least one first material and thereby produce a suitable hydrophobicity of the first material.

The present application therefore provides, in a preferred embodiment, the process of the invention in which a hydrophobizing agent is added in step (A).

In a preferred embodiment, a hydrophobizing agent of the general formula (I)

A-Z

(I)

which binds to the at least one first material, where A is selected from among linear or branched C<sub>3</sub>-C<sub>30</sub>-alkyl, C<sub>3</sub>-C<sub>30</sub>-heteroalkyl, optionally substituted C<sub>6</sub>-C<sub>30</sub>-aryl, optionally substituted C<sub>6</sub>-C<sub>30</sub>-heteroalkyl, C<sub>6</sub>-C<sub>30</sub>-aralkyl and

Z is a group by means of which the compound of the general formula (I) binds to the at least one hydrophobic material, is added in step (A) of the process of the invention.

In a particularly preferred embodiment, A is a linear or branched C<sub>4</sub>-C<sub>12</sub>-alkyl, very particularly preferably a linear C<sub>4</sub>-C<sub>8</sub>-alkyl. Heteroatoms which may be present according to the invention are selected from among N, O, P, S and halogens such as F, Cl, Br and I.

In a further preferred embodiment, A is preferably a linear or branched, preferably linear, C<sub>6</sub>-C<sub>20</sub>-alkyl. Preference is also given to A being a branched C<sub>6</sub>-C<sub>14</sub>-alkyl in which the at least one substituent, preferably having from 1 to 6 carbon atoms, is preferably present in the 2 position, for example 2-ethylhexyl and/or 2-propylheptyl.

In a further particularly preferred embodiment, Z is selected from the group consisting of anionic groups —(X)<sub>n</sub>—PO<sub>3</sub><sup>2-</sup>, —(X)<sub>n</sub>—PO<sub>2</sub>S<sup>2-</sup>, —(X)<sub>n</sub>—POS<sub>2</sub><sup>2-</sup>, —(X)<sub>n</sub>—PS<sub>3</sub><sup>2-</sup>, —(X)<sub>n</sub>—PS<sub>2</sub><sup>-</sup>, —(X)<sub>n</sub>—POS<sup>-</sup>, —(X)<sub>n</sub>—PO<sub>2</sub><sup>-</sup>, —(X)<sub>n</sub>—PO<sub>3</sub><sup>2-</sup>, —(X)<sub>n</sub>—CO<sub>2</sub><sup>-</sup>, —(X)<sub>n</sub>—CS<sub>2</sub><sup>-</sup>, —(X)<sub>n</sub>—COS<sup>-</sup>, —(X)<sub>n</sub>—C(S)NHOH, —(X)<sub>n</sub>—S<sup>-</sup>, where X is selected from the group consisting of O, S, NH, CH<sub>2</sub> and n=0, 1 or 2, with, if appropriate, cations selected from the group consisting of hydrogen, NR<sub>4</sub><sup>+</sup> where the radicals R are each, independently of one another, hydrogen or C<sub>1</sub>-C<sub>8</sub>-alkyl, alkali or alkaline earth metals. The anions mentioned and the corresponding cations form, according to the invention, uncharged compounds of the general formula (I).

If n=2 in the formulae mentioned, two identical or different, preferably identical, groups A are bound to a group Z.

In a particularly preferred embodiment, use is made of compounds selected from the group consisting of xanthates A—O—CS<sub>2</sub><sup>-</sup>, dialkyldithiophosphates (A—O)<sub>2</sub>—PS<sub>2</sub><sup>-</sup>, dialkyldithiophosphinates (A)<sub>2</sub>—PS<sub>2</sub><sup>-</sup> and mixtures thereof, where the radicals A are each, independently of one another, a linear or branched, preferably linear, C<sub>6</sub>-C<sub>20</sub>-alkyl, for example n-octyl, or a branched C<sub>6</sub>-C<sub>14</sub>-alkyl, with the branch preferably being in the 2 position, for example 2-ethylhexyl and/or 2-propylheptyl. In these compounds, counterions present are preferably cations selected from the group consisting of hydrogen, NR<sub>4</sub><sup>+</sup> where the radicals R are each, independently of one another, hydrogen or C<sub>1</sub>-C<sub>8</sub>-alkyl, alkali or alkaline earth metals, in particular sodium or potassium.

Very particularly preferred compounds of the general formula (I) are selected from the group consisting of sodium or potassium n-octylxanthate, sodium or potassium butylxanthate, sodium or potassium di-n-octyldithiophosphinate, sodium or potassium di-n-octyldithiophosphate, and mixtures of these compounds.

In the case of noble metals, for example Au, Pd, Rh, etc., particularly preferred surface-active substances are mono-thiols, dithiols and trithiols or 8-hydroxyquinolines, for example as described in EP 1200408 B1.

In the case of metal oxides, for example FeO(OH), Fe<sub>3</sub>O<sub>4</sub>, ZnO, etc., carbonates, for example azurite [Cu(CO<sub>3</sub>)<sub>2</sub>(OH)<sub>2</sub>], malachite [Cu<sub>2</sub>[(OH)<sub>2</sub>CO<sub>3</sub>]], particularly preferred hydrophobizing agents are octylphosphonic acid (OPA),

(EtO)<sub>3</sub>Si-A, (MeO)<sub>3</sub>Si-A, where A has the abovementioned meanings. In a preferred embodiment of the process of the invention, no hydroxylates are used as hydrophobizing agent for modifying metal oxides.

5 In the case of metal sulfides, for example Cu<sub>2</sub>S, MoS<sub>2</sub>, etc., particularly preferred hydrophobizing agents are mono-thiols, dithiols and trithiols or xanthogenates.

In a further preferred embodiment of the process of the invention, Z is —(X)<sub>n</sub>—CS<sub>2</sub><sup>-</sup>, —(X)<sub>n</sub>—PO<sub>2</sub><sup>-</sup> or —(X)<sub>n</sub>—S<sup>-</sup> where X is O and n is 0 or 1 and a cation selected from among hydrogen, sodium or potassium. Very particularly preferred hydrophobizing agents are 1-octanethiol, potassium n-octylxanthate, potassium butylxanthate, octylphosphonic acid and di(n-octyl) thionocarbamate (a compound of the formula (II))



The addition of at least one abovementioned hydrophobizing agent in step (A) of the process of the invention is preferably carried out when the hydrophobicity of the at least one first material is not sufficiently high, particularly preferably when the at least one first material is selected from among FeCu<sub>2</sub>, CuS<sub>2</sub>.

35 Providing the mixture of the at least one hydrocarbon and, if appropriate, the at least one hydrophobizing agent in step (A) of the process of the invention can occur by all methods known to those skilled in the art. Step (A) can be carried out in bulk or in dispersion, preferably in suspension, particularly preferably in aqueous suspension.

In an embodiment of the process of the invention, step (A) is carried out in bulk, i.e. in the absence of a dispersion medium.

40 For example, the mixture to be treated and the at least one hydrocarbon or hydrocarbon mixture and, if appropriate, at least one hydrophobizing agent are combined and mixed in the appropriate amounts without a further dispersion medium. Suitable mixing apparatuses are known to those skilled in the art, for example mills such as a ball mill.

45 In a further preferred embodiment, step (A) is carried out in a dispersion, preferably in suspension. As dispersion media, it is possible to use all dispersion media in which the mixture in step (A) is not completely soluble. Suitable dispersion media for preparing the slurry or dispersion in step (A) of the process of the invention are selected from the group consisting of water, water-soluble organic compounds, for example alcohols having from 1 to 4 carbon atoms, and mixtures thereof.

50 In a particularly preferred embodiment, the dispersion medium in step (A) is water.

The solids content of the dispersion obtained in step (A) is generally from 40 to 80% by weight, preferably from 50 to 70% by weight, in each case based on the total mixture.

55 In another embodiment, the solids content of the dispersion obtained in step (A) is generally from 0.1 to 99.5% by weight, preferably from 5 to 50% by weight, in each case based on the total mixture.

Step (A) of the process of the invention is generally carried out at a temperature of from 1 to 80° C., preferably from 20 to 40° C., particularly preferably at ambient temperature.

## Step (B):

The optional step (B) of the process of the invention comprises addition of at least one dispersion medium to the mixture obtained in step (A) in order to obtain a dispersion.

The mixture obtained in step (A) comprises, in one embodiment when step (A) is carried out in bulk, at least one first material, at least one second material and at least one third material and also at least one hydrocarbon and, if appropriate, at least one hydrophobizing agent. If step (A) is carried out in bulk, step (B) of the process of the invention is carried out, i.e. at least one suitable dispersion medium is added to the mixture obtained in step (A) in order to obtain a dispersion.

In the embodiment in which step (A) of the process of the invention is carried out in dispersion, it is not absolutely necessary to carry out step (B). However, even in this embodiment, preference is given to carrying out step (B), i.e. further dispersion medium is added in order to obtain, in step (B), a dispersion which has a lower solids content than the dispersion in step (A).

Suitable dispersion media are all dispersion media which have already been mentioned in respect of step (A). In a particularly preferred embodiment, the dispersion medium in step (B) is water.

Thus, in step (B), either the mixture present in bulk from step (A) is converted into a dispersion or the mixture which is already present in dispersion from step (A) is converted into a dispersion having a lower solids content by addition of dispersion medium.

In general, the amount of dispersion medium added in step (A) and/or step (B) can, according to the invention, be selected so that a dispersion which is readily stirrable and/or flowable is obtained. In a preferred embodiment, the solids content of the dispersion obtained in step (B) of the process of the invention is from 0.5 to 50% by weight, preferably from 10 to 40% by weight, more preferably from 10 to 30% by weight, still more preferably 20 to 30% by weight, particularly preferably from 22 to 28% by weight, in each case based on the total dispersion.

In a preferred embodiment of the process of the invention, step (B) is carried out since an aqueous dispersion having a high solids content, as indicated above, is preferably produced in step (A) and this is preferably converted in step (B) into a dispersion which has a lower solids content, as indicated above, in order to be used in step (C) of the process of the invention.

The addition of dispersion medium in step (B) of the process of the invention can, according to the invention, be carried out by all methods known to those skilled in the art.

In preferred embodiments, the mixture of step (A) or, if step (B) is carried out, the dispersion obtained from step (B) can be mixed vigorously such that a specific energy in an amount of at least 1 kWh/m<sup>3</sup>, such as 1 to 300 kWh/m<sup>3</sup>, preferably 1 to 50 kWh/m<sup>3</sup> is introduced into the mixture prior to step (C). In order to accomplish the introduction of such an amount of specific energy, mixing at a specific power of at least 10 kW/m<sup>3</sup>, such as 10 to 3500 kW/m<sup>3</sup>, preferably 10 to 1000 kW/m<sup>3</sup> can be carried out. Mixing is carried out for a period of 5 minutes or less, 15 minutes or less, 30 minutes or less, 1 hour or less, 6 hours or less or 12 hours or less. The time of mixing and the specific power employed for mixing are adjusted such that the desired amount of specific energy can be introduced.

The energy can be introduced into the mixture or dispersion by different means. Typically it is done by a stirred vessel that may contain baffles to render the energy uptake more efficient. Also a common mean to keep a slurry

homogeneous and introducing mixing energy is to circulate the content of a vessel may it be stirred or not by a circulating pump e.g. a centrifugal pump. Other means are milling aggregates like ball mills or any type of stirred ball mills. Also the use of rotor stator mixing devices is possible. Provided the correct amount of energy can be introduced the turbulent flow of the dispersion through a pipe conveyed by pumps or by gravity will also yield the required agglomeration. Static mixers and counter current flow mixers are another way to introduce shear energy into the flowing dispersion of the first type particles, the second type particles and the magnet type particles.

The specific energy (i.e. the amount of energy per volume) introduced is calculated by dividing the stirring power by the suspension volume multiplied by the treatment time [h]. The stirring power is calculated (e.g. for a stirred vessel) from the formula

$$P = \rho Ne n^3 d^6$$

with  $\rho$ =density [kg/m<sup>3</sup>],  $n$ =rotational speed of stirrer [sec<sup>-1</sup>],  $d$ =stirrer diameter,  $Ne$ =Newton number [-].

The Newton no. is obtained from experimentally determined Reynolds no. and published correlations between Newton and Reynolds no. for different stirrer geometries (J. H. Rushton, E. W. Costich, H. J. Everett, Power Characteristics of mixing impellers, Part I, Chem. Eng. Progr. 46 (8) 395-404 (1950) and J. H. Rushton, E. W. Costich, H. J. Everett, Power Characteristics of mixing impellers, Part II, Chem. Eng. Progr. 46 (9) 467-476 (1950) for propeller with ring and radial flow impeller; J. G. van de Vusse Mixing by agitation of miscible liquids, Part I, Chem. Eng. Sci. 4/178-200 (1955) and J. G. van de Vusse Mixing by agitation of miscible liquids, Part II, Chem. Eng. Sci. 4/209-220 (1955) for pitched blade turbines).

## Step (C):

Step (C) of the process of the invention comprises treatment of the dispersion from step (A) or (B) with at least one hydrophobic magnetic particle so that the at least one first material and the at least one magnetic particle agglomerate.

In step (C) of the process of the invention, it is possible to use all magnetic substances and materials known to those skilled in the art. In a preferred embodiment, the at least one magnetic particle is selected from the group consisting of magnetic metals, for example iron, cobalt, nickel and mixtures thereof, ferromagnetic alloys of magnetic metals, for example NdFeB, SmCo and mixtures thereof, magnetic iron oxides, for example magnetite, maghemite, cubic ferrites of the general formula (III)



(III)

where

$M$  is selected from among Co, Ni, Mn, Zn and mixtures thereof and

$x$  is  $\leq 1$ ,

hexagonal ferrites, for example barium or strontium ferrite  $MFe_6O_19$  where  $M=Ca, Sr, Ba$ , and mixtures thereof. The magnetic particles can additionally have an outer layer, for example of  $SiO_2$ .

In a particularly preferred embodiment of the present patent application, the at least one magnetic particle is magnetite or cobalt ferrite  $Co^{2+}xFe^{2+}Fe^{3+}O_4$  where  $x \leq 1$ .

In a further preferred embodiment, the at least one magnetic particle is hydrophobized on the surface by means of at least one hydrophobic compound. The hydrophobic compound is preferably selected from among compounds of the general formula (IV)



(IV),

## 11

wherein each B is independently selected from among linear or branched  $C_1$ - $C_{30}$ -alkyl,  $C_1$ - $C_{30}$ -heteroalkyl, optionally substituted  $C_6$ - $C_{30}$ -aryl, optionally substituted  $C_6$ - $C_{30}$ -heteroalkyl,  $C_6$ - $C_{30}$ -aralkyl; and each Y is independently selected as a group by means of which the compound of the general formula (III) binds to the at least one magnetic particle; each e is the integer 1, 2, 3, 4, 5, 6, 7, 8, 9 or 10; each f is the integer 1, 2, 3, 4, 5, 6, 7, 8, 9 or 10; and each g is the integer 1, 2, 3, 4, 5, 6, 7, 8, 9 or 10 to 100.

In a particularly preferred embodiment, B is a linear or branched  $C_6$ - $C_{18}$ -alkyl, preferably linear  $C_8$ - $C_{12}$ -alkyl and very particularly preferably a linear  $C_{12}$ -alkyl.

In a further particularly preferred embodiment, Y is selected from the group consisting of  $-(X)_p-Si(R^2)_3$ ,  $-(X)_p-SiH(R^2)_2$ ,  $-(X)_p-SiH_2R^2$  wherein each  $R^2$  is independently selected from F, Cl, Br, I or OH; and anionic groups such as



wherein each X is independently O, S, NH, or  $CH_2$  and p is 0, 1 or 2.

Very particularly preferred hydrophobizing agents of the general formula (IV) are silicon-based oils or siloxanes resulting from in-situ hydrolysis of dodecyl- or other alkyl-trichlorosilanes or alkyltrialkoxysilanes; phosphonic acids, for example octylphosphonic acid; carboxylic acids; for example lauric acid, oleic acid or stearic acid; partly polymerized siloxanes (also known as silicon oils), or mixtures thereof.

Suitable hydrophobizing agent are compounds as disclosed in WO 2012/028701, WO 2015/110555 or WO 2012/140065.

Further preferred hydrophobizing agents are mono-, oligo- or polysiloxanes with free OH groups, such as the compounds of formula (IVa), (IVb) and (IVc) or derivatives thereof.



(IVa)

## 12

-continued



(IVb)



(IVc)

wherein each r, s, t, and u is independently an integer from 1 to 100, and each  $R^3$  is independently a straight or branched  $C_1$ - $C_{12}$  alkyl group.

In formula (IVc), \* denotes a bonding to further moieties comprising  $-SiOR^4$  and wherein  $R^4$  is selected from hydrogen, linear or branched, optionally substituted  $C_1$ - $C_{30}$ -alkyl, linear or branched, optionally substituted  $C_2$ - $C_{30}$ -alkenyl, linear or branched, optionally substituted  $C_2$ - $C_{30}$ -alkynyl, optionally substituted  $C_3$ - $C_{20}$ -cycloalkyl, optionally substituted  $C_3$ - $C_{20}$ -cycloalkenyl, optionally substituted  $C_1$ - $C_{20}$ -heteroalkyl, optionally substituted  $C_5$ - $C_{22}$ -aryl, optionally substituted  $C_6$ - $C_{23}$ -alkylaryl, optionally substituted  $C_6$ - $C_{23}$ -arylalkyl or optionally substituted  $C_5$ - $C_{22}$ -heteroaryl.

In a preferred embodiment, the hydrophobizing agents of formula (IVa), (IVb) or (IVc) have a molecular weight from about 250 to about 200000 g/mol, preferably from about 250 to about 20000 g/mol and particularly preferably from about 300 to about 5000 g/mol.

According to a preferred embodiment, the hydrophobizing agent is a compound of the general formulas (V), (Va), (Vb), (Vc) or derivatives thereof



(Va)



(Vb)



(Vc)

wherein each  $R^5$  is independently selected from hydrogen, linear or branched, optionally substituted  $C_1$ - $C_{30}$ -alkyl, linear or branched, optionally substituted  $C_2$ - $C_{30}$ -alkenyl, linear or branched, optionally substituted  $C_2$ - $C_{30}$ -alkynyl, optionally substituted  $C_3$ - $C_{20}$ -cycloalkyl, optionally substituted  $C_1$ - $C_{20}$ -heteroalkyl, optionally substituted  $C_5$ - $C_{22}$ -aryl, optionally substituted  $C_6$ - $C_{23}$ -alkylaryl, optionally substituted  $C_6$ - $C_{23}$ -arylalkyl or optionally substituted  $C_5$ - $C_{22}$ -heteroaryl;

each  $R^6$  is independently selected from hydrogen, linear or branched, optionally substituted  $C_1$ - $C_{30}$ -alkyl, linear or branched, optionally substituted  $C_2$ - $C_{30}$ -alkenyl, linear or branched, optionally substituted  $C_2$ - $C_{30}$ -alkynyl, optionally substituted  $C_3$ - $C_{20}$ -cycloalkyl, optionally substituted  $C_3$ - $C_{20}$ -cycloalkenyl, optionally substituted  $C_1$ - $C_{20}$ -heteroalkyl, optionally substituted  $C_5$ - $C_{22}$ -aryl, optionally substituted  $C_6$ - $C_{23}$ -alkylaryl, optionally substituted  $C_6$ - $C_{23}$ -arylkyl or optionally substituted  $C_5$ - $C_{22}$ -heteroaryl, and the integer  $r$  is as described above and  $v$  is the integer 1, 2 or 3.

Preference is given to the radicals  $R^5$  each being, independently of one another, linear or branched, optionally substituted  $C_1$ - $C_{30}$ -alkyl, particularly preferably  $C_1$ - $C_{20}$ -alkyl, very particularly preferably  $C_4$ - $C_{12}$ -alkyl. In a preferred embodiment,  $R^5$  is linear or branched, unsubstituted  $C_1$ - $C_{30}$ -alkyl, particularly preferably  $C_1$ - $C_{20}$ -alkyl or very particularly preferably  $C_4$ - $C_{12}$ -alkyl. Examples of linear or branched  $C_4$ - $C_{12}$ -alkyl radicals are butyl, in particular, n-butyl, isobutyl, tert-butyl; pentyl, in particular n-pentyl, isopentyl, tert-pentyl; hexyl, in particular n-hexyl, isohexyl, tert-hexyl, heptyl; in particular n-heptyl, isoheptyl, tert-heptyl; octyl in particular n-octyl, isoctyl, tert-octyl; nonyl, in particular n-nonyl, isononyl, tert-nonyl, decyl, in particular n-decyl, isodecyl, tert-decyl, undecyl, in particular n-undecyl, isoundecyl, tert-undecyl, or dodecyl, in particular n-dodecyl; isododecyl or tert-dodecyl.

Further preference is given to the radicals  $R^5$  each being, independently of one another, linear or branched, optionally substituted  $C_2$ - $C_{30}$ -alkenyl, particularly preferably  $C_2$ - $C_{20}$ -alkenyl, very particularly preferably or  $C_2$ - $C_{12}$ -alkenyl. Examples of alkenyl radicals which are particularly preferred according to the invention are ethenyl (vinyl), propenyl, in particular n-propenyl, isopropenyl, butenyl, in particular n-butenyl, isobutetyl, tert-butenyl, pentenyl, in particular n-pentenyl, isopentenyl, tert-pentenyl, hexenyl, in particular n-hexenyl, isohexenyl, tert-hexenyl, heptenyl, in particular n-heptenyl, isoheptenyl, tert-heptenyl, octenyl, in particular n-octenyl, isoctenyl, tert-octenyl, nonenyl, in particular n-nonenyl, isononenyl, tert-nonenyl, decenyl, in particular n-deceny, isodeceny, tert-deceny, undecenyl, in particular n-undeceny, isoundeceny, tert-undeceny, or dodeceny, in particular n-dodeceny, isododeceny and tert-dodeceny.

Further preference is given to the radicals  $R^5$  each being, independently of one another, linear or branched, optionally substituted  $C_2$ - $C_{30}$ -alkynyl, particularly preferably  $C_2$ - $C_{20}$ -alkynyl, very particularly preferably  $C_2$ - $C_{12}$ -alkynyl. Examples of alkynyl radicals which are particularly preferred according to the invention are ethynyl, propynyl, in particular n-propynyl, isopropynyl, butynyl, in particular n-butyne, isobutynyl, tert-butyne, pentynyl, in particular n-pentyne, isopentyne, tert-pentyne, hexynyl, in particular n-hexyne, isohexyne, tert-hexyne, heptynyl, in particular n-heptynyl, isoheptynyl, tert-heptynyl, octynyl, in particular n-octyne, isoctyne, tert-octyne, nonyne, in particular n-nonyne, isonynyne, tert-nonyne, decyne, in particular n-deceny, isodeceny, tert-deceny, undeceny, in particular n-undeceny, isoundeceny, tert-undeceny, or dodeceny, in particular n-dodeceny, isododeceny and tert-dodeceny.

Further preference is given to the radicals  $R^5$  each being, independently of one another, optionally substituted  $C_3$ - $C_{20}$ -cycloalkyl, particularly preferably  $C_3$ - $C_{12}$ -cycloalkyl, very particularly preferably  $C_3$ - $C_6$ -cycloalkyl, such as cyclopropyl, cyclobutyl, cyclopentyl or cyclohexyl.

Further preference is given to the radicals  $R^5$  each being, independently of one another, optionally substituted  $C_3$ - $C_{20}$ -

cycloalkenyl, particularly preferably  $C_3$ - $C_{12}$ -cycloalkenyl, very particularly preferably  $C_3$ - $C_6$ -cycloalkenyl such as cyclopropenyl, cyclobutenyl, cyclopentenyl or cyclohexenyl.

Further preference is given to the radicals  $R^5$  each being, independently of one another, optionally substituted  $C_1$ - $C_{20}$ -heteroalkyl, particularly preferably  $C_1$ - $C_{12}$ -heteroalkyl. The heteroalkyl radicals present according to the invention are derived from the abovementioned alkyl radicals, with at least one carbon atom being replaced by a heteroatom selected from among N, O, P and S.

Further preference is given to the radicals  $R^5$  each being, independently of one another, optionally substituted  $C_5$ - $C_{22}$ -aryl, particularly preferably  $C_5$ - $C_{12}$ -aryl. Examples of aryl radicals which are preferred according to the invention are phenyl, naphthyl or biaryl.

Further preference is given to the radicals  $R^5$  each being, independently of one another, optionally substituted  $C_6$ - $C_{23}$ -alkylaryl, particularly preferably  $C_6$ - $C_{13}$ -alkylaryl. An example of an alkylaryl radical which is preferred according to the invention is benzyl.

Further preference is given to the radicals  $R^5$  each being, independently of one another, optionally substituted  $C_6$ - $C_{23}$ -arylalkyl, particularly preferably  $C_6$ - $C_{13}$ -arylalkyl. Examples of arylalkyl radicals which are preferred according to the invention are tolyl, xylyl, propylbenzyl or hexylbenzyl.

Further preference is given to the radicals  $R^5$  each being, independently of one another, optionally substituted  $C_5$ - $C_{22}$ -heteroaryl, particularly preferably  $C_5$ - $C_{12}$ -heteroaryl.

The abovementioned radicals  $R^5$  can optionally be substituted. Suitable substituents are, for example, selected from among amino, amido, imido, hydroxyl, ether, aldehyde, keto, carboxylic acid, thiol, thioether, hydroxamate and carbamate groups. The abovementioned radicals  $R^5$  can be mono- or poly-substituted. In the case of multiple substitutions, one substituent group can be present a plurality of times or various functional groups are simultaneously present. The radicals mentioned for  $R^5$  can also be monosubstituted or polysubstituted by the abovementioned alkyl, alkynyl, alkylaryl, aryl, alkylaryl, arylalkyl, heteroalkyl or heteroaryl radicals.

Very particularly preferred radicals  $R^5$  are octyl, in particular n-octyl; hexyl, in particular n-hexyl; and/or butyl, in particular n-butyl; decyl, in particular n-decyl; or dodecyl, in particular n-dodecyl.

Preference is given to the radicals  $R^6$  each being, independently of one another, hydrogen, linear or branched, optionally substituted  $C_1$ - $C_{30}$ -alkyl, particularly preferably  $C_1$ - $C_{20}$ -alkyl, very particularly preferably  $C_1$ - $C_{12}$ -alkyl. In a preferred embodiment,  $R^6$  is linear or branched, unsubstituted  $C_1$ - $C_{30}$ -alkyl, particularly preferably  $C_1$ - $C_{20}$ -alkyl, or very particularly preferably  $C_1$ - $C_{12}$ -alkyl. Examples of linear or branched  $C_1$ - $C_{12}$ -alkyl radicals are methyl, ethyl, propyl, in particular n-propyl, isopropyl, butyl, in particular n-butyl, isobutyl, tert-butyl, pentyl, in particular n-pentyl, isopentyl, tert-pentyl, hexyl, in particular n-hexyl, isohexyl, tert-hexyl, heptyl, in particular n-heptyl, isoheptyl, tert-heptyl, octyl, in particular n-octyl, isoctyl, tert-octyl, nonyl, in particular n-nonyl, isonynyl, tert-nonyl, decyl, in particular n-decyl, isodecyl, tert-decyl, undecyl, in particular n-undecyl, isoundecyl, tert-undecyl, or dodecyl, in particular n-dodecyl, isododecyl or tert-dodecyl.

Further preference is given to the radicals  $R^6$  each being, independently of one another, linear or branched, optionally substituted  $C_2$ - $C_{30}$ -alkenyl, particularly preferably  $C_2$ - $C_{20}$ -alkenyl and very particularly preferably  $C_2$ - $C_{12}$ -alkenyl.

Examples of alkynyl radicals which are particularly preferred according to the invention are ethenyl (vinyl), propenyl, in particular n-propenyl, isopropenyl, butenyl, in particular n-butenyl, isobut enyl, tert-but enyl, pentenyl, in particular n-pentenyl, isopentenyl, tert-pentenyl, hexenyl, in particular n-hexenyl, isohexenyl, tert-hexenyl, heptenyl, in particular n-heptenyl, isoheptenyl, tert-heptenyl, octenyl, in particular n-octenyl, isoctenyl, tert-octenyl, nonenyl, in particular n-nonenyl, isononenyl, tert-nonenyl, decenyl, in particular n-decenyl, isodecenyl, tert-decenyl, undecenyl, in particular n-undecenyl, isoundecenyl, tert-undecenyl, or dodecenyl, in particular n-dodecenyl, isododecenyl or tert-dodecenyl.

Further preference is given to the radicals R<sup>6</sup> each being, independently of one another, linear or branched, optionally substituted C<sub>2</sub>-C<sub>30</sub>-alkynyl, particularly preferably C<sub>2</sub>-C<sub>20</sub>-alkynyl or very particularly preferably C<sub>2</sub>-C<sub>12</sub>-alkynyl. Examples of alkynyl radicals which are particularly preferred according to the invention are ethynyl, propynyl, in particular n-propynyl, isopropynyl, butynyl, in particular n-butynyl, isobutynyl, tert-butynyl, pentynyl, in particular n-pentynyl, isopentynyl, tert-pentynyl, hexynyl, in particular n-hexynyl, isohexynyl, tert-hexynyl, heptynyl, in particular n-heptynyl, isoheptynyl, tert-heptynyl, octynyl, in particular n-octynyl, isoctynyl, tert-octynyl, nonynyl, in particular n-nonyl, isononyl, tert-nonyl, decynyl, in particular n-decynyl, isodecynyl, tert-decynyl, undecynyl, in particular n-undecynyl, isoundecynyl, tert-undecynyl, or dodecynyl, in particular n-dodecynyl, isododecynyl or tert-dodecynyl.

Further preference is given to the radicals R<sup>6</sup> each being, independently of one another, optionally substituted C<sub>3</sub>-C<sub>20</sub>-cycloalkyl, particularly preferably C<sub>3</sub>-C<sub>12</sub>-cycloalkyl and particularly preferably C<sub>3</sub>-C<sub>6</sub>-cycloalkyl, for example cyclopropyl, cyclobutyl, cyclopentyl or cyclohexyl.

Further preference is given to the radicals R<sup>6</sup> each being, independently of one another, optionally substituted C<sub>3</sub>-C<sub>20</sub>-cycloalkenyl, particularly preferably C<sub>3</sub>-C<sub>12</sub>-cycloalkenyl and very particularly preferably C<sub>3</sub>-C<sub>6</sub>-cycloalkenyl, for example cyclopropenyl, cyclobut enyl, cyclopentenyl or cyclohexenyl.

Further preference is given to the radicals R<sup>6</sup> each being, independently of one another, optionally substituted C<sub>1</sub>-C<sub>20</sub>-heteroalkyl, particularly preferably C<sub>4</sub>-C<sub>12</sub>-heteroalkyl. The heteroalkyl radicals which are present according to the invention are derived from the abovementioned alkyl radicals, with at least one carbon atom being replaced by a heteroatom selected from among N, O, P and S.

Further preference is given to the radicals R<sup>6</sup> each being, independently of one another, optionally substituted C<sub>5</sub>-C<sub>22</sub>-aryl, particularly preferably C<sub>5</sub>-C<sub>22</sub>-aryl. Examples of aryl radicals which are preferred according to the invention are phenyl, naphthyl or biaryls.

Further preference is given to the radicals R<sup>6</sup> each being, independently of one another, optionally substituted C<sub>6</sub>-C<sub>23</sub>-alkylaryl, particularly preferably C<sub>6</sub>-C<sub>13</sub>-alkylaryl. An example of an alkylaryl radical which is preferred according to the invention is benzyl.

Further preference is given to the radicals R<sup>6</sup> each being, independently of one another, optionally substituted C<sub>6</sub>-C<sub>23</sub>-arylalkyl and particularly preferably C<sub>6</sub>-C<sub>13</sub>-arylalkyl. Examples of arylalkyl radicals which are preferred according to the invention are tolyl, xylyl, propylbenzyl or hexylbenzyl.

Further preference is given to the radicals R<sup>6</sup> each being, independently of one another, optionally substituted C<sub>5</sub>-C<sub>2</sub>-heteroaryl and particularly preferably C<sub>5</sub>-C<sub>12</sub>-heteroaryl.

The abovementioned radicals R<sup>6</sup> may optionally be substituted. Suitable substituents are, for example, selected from among amino, amido, imido, hydroxy, ether, aldehyde, keto, carboxylic acid, thiol, thioether, hydroxamate and carbamate groups. The abovementioned radicals R<sup>6</sup> can be mono- or poly substituted. In the case of multiple substitutions, one substituent can be present a plurality of times or various functional groups are simultaneously present. The radicals mentioned for R<sup>6</sup> can also be monosubstituted or polysubstituted by the abovementioned alkyl, alkenyl, alkynyl, aryl, alkylaryl, arylalkyl, heteroalkyl or heteroaryl radicals.

In another preferred embodiment, the at least one hydrophobizing agent is selected from the group consisting of (NaO)(CH<sub>3</sub>)Si(OH)<sub>2</sub>, (NaO)(C<sub>2</sub>H<sub>5</sub>)Si(OH)<sub>2</sub>, (NaO)(C<sub>5</sub>H<sub>11</sub>)Si(OH)<sub>2</sub>, (NaO)(C<sub>8</sub>H<sub>17</sub>)Si(OH)<sub>2</sub>, (KO)(CH<sub>3</sub>)Si(OH)<sub>2</sub>, (KO)(C<sub>2</sub>H<sub>5</sub>)Si(OH)<sub>2</sub>, (KO)(C<sub>5</sub>H<sub>11</sub>)Si(OH)<sub>2</sub>, (KO)(C<sub>8</sub>H<sub>17</sub>)Si(OH)<sub>2</sub>, (NH<sub>4</sub>O)(CH<sub>3</sub>)Si(OH)<sub>2</sub>, (NH<sub>4</sub>O)(C<sub>2</sub>H<sub>5</sub>)Si(OH)<sub>2</sub>, (NH<sub>4</sub>O)(C<sub>5</sub>H<sub>11</sub>)Si(OH)<sub>2</sub>, (NH<sub>4</sub>O)(C<sub>8</sub>H<sub>17</sub>)Si(OH)<sub>2</sub>, (NaO)<sub>2</sub>(CH<sub>3</sub>)Si(OH), (NaO)<sub>2</sub>(C<sub>2</sub>H<sub>5</sub>)Si(OH), (NaO)<sub>2</sub>(C<sub>5</sub>H<sub>11</sub>)Si(OH), (NaO)<sub>2</sub>(C<sub>8</sub>H<sub>17</sub>)Si(OH), (NaO)<sub>2</sub>(C<sub>2</sub>H<sub>5</sub>)Si(OH), (KO)<sub>2</sub>(CH<sub>3</sub>)Si(OH), (KO)<sub>2</sub>(C<sub>2</sub>H<sub>5</sub>)Si(OH), (KO)<sub>2</sub>(C<sub>5</sub>H<sub>11</sub>)Si(OH), (KO)<sub>2</sub>(C<sub>8</sub>H<sub>17</sub>)Si(OH), (NH<sub>4</sub>O)<sub>2</sub>(CH<sub>3</sub>)Si(OH), (NH<sub>4</sub>O)<sub>2</sub>(C<sub>2</sub>H<sub>5</sub>)Si(OH), (NH<sub>4</sub>O)<sub>2</sub>(C<sub>5</sub>H<sub>11</sub>)Si(OH), (NH<sub>4</sub>O)<sub>2</sub>(C<sub>8</sub>H<sub>17</sub>)Si(OH), (NaO)<sub>3</sub>(CH<sub>3</sub>)Si, (NaO)<sub>3</sub>(C<sub>2</sub>H<sub>5</sub>)Si, (NaO)<sub>3</sub>(C<sub>5</sub>H<sub>11</sub>)Si, (NaO)<sub>3</sub>(C<sub>8</sub>H<sub>17</sub>)Si, (KO)<sub>3</sub>(CH<sub>3</sub>)Si, (KO)<sub>3</sub>(C<sub>2</sub>H<sub>5</sub>)Si, (KO)<sub>3</sub>(C<sub>5</sub>H<sub>11</sub>)Si, (KO)<sub>3</sub>(C<sub>8</sub>H<sub>17</sub>)Si, (NH<sub>4</sub>O)<sub>3</sub>(CH<sub>3</sub>)Si, (NH<sub>4</sub>O)<sub>3</sub>(C<sub>2</sub>H<sub>5</sub>)Si, (NH<sub>4</sub>O)<sub>3</sub>(C<sub>5</sub>H<sub>11</sub>)Si, (NH<sub>4</sub>O)<sub>3</sub>(C<sub>8</sub>H<sub>17</sub>)Si, (NaO)(CH<sub>3</sub>)<sub>2</sub>Si(OH), (NaO)(C<sub>2</sub>H<sub>5</sub>)<sub>2</sub>Si(OH), (KO)(CH<sub>3</sub>)<sub>2</sub>Si(OH), (KO)(C<sub>2</sub>H<sub>5</sub>)<sub>2</sub>Si(OH), (NaO)<sub>2</sub>(CH<sub>3</sub>)<sub>2</sub>Si, (NaO)<sub>2</sub>(C<sub>2</sub>H<sub>5</sub>)<sub>2</sub>Si, (KO)<sub>2</sub>(CH<sub>3</sub>)<sub>2</sub>Si, (KO)<sub>2</sub>(C<sub>2</sub>H<sub>5</sub>)<sub>2</sub>Si, Ca<sup>2+</sup>[(O<sup>-</sup>)(CH<sub>3</sub>)Si(OH)]<sub>2</sub>, Ca<sup>2+</sup>[(O<sup>-</sup>)(C<sub>2</sub>H<sub>5</sub>)Si(OH)]<sub>2</sub>, Ca<sup>2+</sup>[(O<sup>-</sup>)(C<sub>5</sub>H<sub>11</sub>)Si(OH)]<sub>2</sub>, Ca<sup>2+</sup>[(O<sup>-</sup>)(C<sub>8</sub>H<sub>17</sub>)Si(OH)]<sub>2</sub>, Ca<sup>2+</sup>[(O<sup>-</sup>)(CH<sub>3</sub>)<sub>2</sub>Si(OH)]<sub>2</sub>, Ca<sup>2+</sup>[(O<sup>-</sup>)(C<sub>2</sub>H<sub>5</sub>)<sub>2</sub>Si(OH)]<sub>2</sub>, Ca<sup>2+</sup>[(O<sup>-</sup>)(C<sub>5</sub>H<sub>11</sub>)<sub>2</sub>Si(OH)], Ca<sup>2+</sup>[(O<sup>-</sup>)(C<sub>8</sub>H<sub>17</sub>)<sub>2</sub>Si(OH)], Ca<sup>2+</sup>[(O<sup>-</sup>)<sub>2</sub>(CH<sub>3</sub>)<sub>2</sub>Si], Ca<sup>2+</sup>[(O<sup>-</sup>)<sub>2</sub>(C<sub>2</sub>H<sub>5</sub>)<sub>2</sub>Si] and combinations thereof.

The treatment of the solution or dispersion with at least one hydrophobic magnetic particle in step (C) of the process of the invention can be effected by all methods known to those skilled in the art.

In a preferred embodiment, the at least one magnetic particle is dispersed in a suitable dispersion medium.

Suitable dispersion media are all dispersion media in which the at least one magnetic particle is not completely soluble. Suitable dispersion media for effecting dispersion in step (C) of the process of the invention are selected from the group consisting of water, water-soluble organic compounds, for example alcohols having from 1 to 4 carbon atoms, for example methanol, ethanol, n-propanol, isopropanol, and mixtures thereof, in particular water and/or isopropanol or water/surfactant mixtures.

In general, the amount of dispersion medium for predisposition of the magnetic particles can, according to the invention, be selected so that a slurry or dispersion which is readily stirrable and/or flowable is obtained. In a preferred embodiment, the amount of mixture to be treated based on the total slurry or dispersion is up to 60% by weight.

The dispersion of the magnetic particles can, according to the invention, be produced by all methods known to those skilled in the art. In a preferred embodiment, the magnetic particles to be dispersed and the appropriate amount of dispersion medium or mixture of dispersion media are combined in a suitable reactor, for example a glass reactor, and stirred by means of apparatuses known to those skilled in the art, for example in a glass tank by means of a

mechanically driven propeller stirrer, for example at a temperature of from 1 to 80° C., preferably at ambient temperature.

In step (C) of the process of the invention, the at least one hydrophobic magnetic particle is generally used in an amount which is sufficient to separate virtually all of the at least one first material from the mixture to be treated. The at least one magnetic particle is preferably used in an at least 10-fold, particularly preferably at least 50-fold, very particularly preferably at least 140-fold, weight excess, based on the amount of the at least one first material in the mixture to be treated, in step (C) of the process of the invention. In another embodiment, the weight ratio of magnetic particles to the sum of ore feed particles typical lies between 1:1000 to 1:1, more preferably between 1:100 and 1:20.

The treatment of the dispersion from step (B) with at least one hydrophobic magnetic particle is generally effected by combining the two components by methods known to those skilled in the art. In a preferred embodiment, a dispersion of the at least one magnetic particle is added to the mixture which has been treated beforehand with at least one hydrocarbon. In a further embodiment, the magnetic particle can be added in solid form to a dispersion of the mixture to be treated. In a further preferred embodiment, the two components are present in dispersed form.

In preferred embodiments, the mixture of step (C) is obtained by introducing mixing energies such that a specific energy in an amount of 0.001 to 10 kWh/m<sup>3</sup> is introduced into the mixture of step (C). In order to accomplish the introduction of such an amount of specific energy, mixing at a specific power of 0.01 to 100 kW/m<sup>3</sup> can be carried out. Mixing is carried out for a period of 5 minutes or less, 15 minutes or less, 30 minutes or less, 1 hour or less, 6 hours or less or 12 hours or less. The time of mixing and the specific power employed for mixing are adjusted such that the desired amount of specific energy can be introduced.

The energy can be introduced into the mixture or dispersion by different means. Typically it is done by a stirred vessel that may contain baffles to render the energy uptake more efficient. Also a common mean to keep a slurry homogeneous and introducing mixing energy is to circulate the content of a vessel may it be stirred or not by a circulating pump e.g. a centrifugal pump. Other means are milling aggregates like ball mills or any type of stirred ball mills. Also the use of rotor stator mixing devices is possible. Provided the correct amount of energy can be introduced the turbulent flow of the dispersion through a pipe conveyed by pumps or by gravity will also yield the required agglomeration. Static mixers and counter current flow mixers are another way to introduce shear energy into the flowing dispersion of the first type particles, the second type particles and the magnet type particles.

Step (C) is generally carried out at a temperature of from 1 to 80° C., preferably from 10 to 30° C., for example ambient temperature.

In step (C), the at least one magnetic particle becomes attached to the at least one first material of the mixture to be treated. The bond between the two components is based on hydrophobic interactions. In a preferred embodiment, little if any hydrophobic interaction occurs between the at least one magnetic particle and the at least one second material. In general, there is no bonding interaction between the at least one magnetic particle and the at least one third material, i.e. the hydrophilic component of the mixture, so that no agglomeration between these components occurs. After step (C), adducts of the at least one first material and the at least one magnetic particle are therefore present in addition to the

at least one second material and the at least one third material in the mixture. The process of the invention thus makes it possible to separate off one material selectively from a mixture comprising at least three materials, where at least two of the three materials have a very similar chemical character in respect of hydrophobicity or affinity to the hydrophobizing agent, the anion present, etc.

Step (D):

Step (D) of the process of the invention comprises separation of the adduct from step (C) from the mixture by application of a magnetic field.

Step (D) can, in a preferred embodiment, be carried out by introducing a permanent magnet into the reactor in which the mixture from step (C) is present. In a preferred embodiment, a dividing wall made of nonmagnetic material, for example the glass wall of the reactor, is present between permanent magnet and the mixture to be treated. In a further preferred embodiment of the process of the invention, an electromagnet which is only magnetic when an electric current flows is used in step (D). Suitable apparatuses are known to those skilled in the art.

Step (D) of the process of the invention can be carried out at any suitable temperature, such as above the melting point and below the boiling point of the dispersent, for example in water from 10 to 60° C.

During step (D), the mixture is preferably stirred continually by means of a suitable stirrer.

In step (D), the adduct from step (C) can, if appropriate, be separated off by all methods known to those skilled in the art, for example by draining off the liquid together with the component of the dispersion which is not held by the magnet from the reactor used for step (D) through the bottom valve or pumping away the components of the dispersion which are not held by the at least one magnet through a hose.

The magnetic separators used can be operated in batch or continuous mode. Typical batch separators are HI-filters, typical continuous separators are of the Jones type, WHIMS (wet high intensity magnetic separators) or magnetic drum separators LIMS or MIMS (low intensity or medium intensity magnetic separators).

Step (E):

The optional step (E) of the process of the invention comprises dissociation of the adducts separated off in step (D) in order to obtain the at least one first material and the at least one magnetic particle separately. In a preferred embodiment of the process of the invention, the dissociation in step (E) is carried out nondestructively, i.e. the individual components present in the dispersion are not altered chemically.

The dissociation can be carried out by all methods known to those skilled in art which are suitable for dissociating the adduct in such a way that the at least one magnetic particle can be recovered in reusable form. In a preferred embodiment, the magnetic particle which has been split off is reused in step (C). In general the dissociation of the agglomerates is achieved by introduction of mixing energy to the suspension of the agglomerates. In a preferred embodiment chemicals are added to this mixture in order to weaken the bonds between the magnetic particles and the one first particles.

In a preferred embodiment, the dissociation in step (C) of the process of the invention is effected by treating the adduct with a substance selected from the group consisting of organic solvents, basic compounds, acidic compounds, oxidants, reducing agents, surface-active compounds and mixtures thereof.

Examples of suitable organic solvents are methanol, ethanol, propanol, for example n-propanol or isopropanol, aro-

matic solvents, for example benzene, toluene, xylenes, ethers, for example diethyl ether, methyl t-butyl ether, ketones, for example acetone, diesel and mixtures thereof. Examples of basic compounds which can be used according to the invention are aqueous solutions of basic compounds, for example aqueous solutions of alkali metal and/or alkaline earth metal hydroxides, for example KOH, NaOH, aqueous ammonia solutions, aqueous solutions of organic amines of the general formula  $R^2_3N$ , where the radicals  $R^2$  are selected independently from the group consisting of  $C_1-C_8$ -alkyl, optionally substituted by further functional groups. In a preferred embodiment, step (D) is effected by addition of aqueous NaOH solution to a pH of 13. The acidic compounds can be mineral acids, for example HCl,  $H_2SO_4$ ,  $HNO_3$  or mixtures thereof, organic acids, for example carboxylic acids. As oxidant, it is possible to use, for example,  $Na_2S_2O_4$  or  $H_2O_2$ , for example as a 30% strength by weight aqueous solution of  $H_2O_2$  (Perhydrol).

Examples of surface-active compounds which can be used according to the invention are nonionic, anionic, cationic and/or zwitterionic surfactants. Preferred surfactants are non-ionic alkoxylated alcohols.

In a preferred embodiment, the adduct of at least one first material and magnetic particle is dissociated by means of an organic solvent, particularly preferably acetone or diesel. This operation can also be aided mechanically. In a preferred embodiment, ultrasound is used for aiding the dissociation step.

In general, the organic solvent is used in an amount which is sufficient to dissociate virtually all of the adduct. In a preferred embodiment, from 2 to 100 ml of the organic solvent are used per gram of adduct of at least one first material and magnetic particle which is to be dissociated.

According to the invention, the at least one first material and the at least one magnetic particle are present as a dispersion in the dissociation reagent mentioned, preferably an organic solvent, after the dissociation.

The at least one magnetic particle is separated off from the dispersion comprising this at least one magnetic particle and the at least one first material by means of a permanent magnet or electromagnet. Details of this separation are analogous to step (D) of the process of the invention.

The first material to be separated off, preferably the metal compound to be separated off, is preferably separated from the organic solvent by distilling off the organic solvent. The first material which can be obtained in this way can be purified by further processes known to those skilled in the art. The solvent can, if appropriate after purification, be recirculated to the process of the invention.

## EXAMPLES

### Example 1: Enriched Mo-Ore

In a buffled beaker 20 g of an enriched solid Mo-ore (19.5 g dry mass), containing 30.0% Mo as Molybdenite ( $MoS_2$ ) and 1.5% Cu mainly as Chalcopyrite ( $CuFeS_2$ ), are provided. The material has a particle size  $d80$  of 30  $\mu m$ . The material was dispersed in 60 g of filtrated river water yielding a solid content of 25 w % (step 1).

To this dispersion 500 mg corresponding to a concentration of 25000 g/t solid of a liquid mixed hydrocarbon having a boiling range of 145-202° C. and a dynamic viscosity of  $1.2 \cdot 10^{-6} m^2/sec$  (20° C.) were added (step 2). Afterwards this dispersion was vigorously mixed with an Ultra Turrax T25 stirrer for 10 min at 10000 rpm (spec. energy input approx. 600 kWh/m<sup>3</sup>) (Step 2a).

Subsequently to this slurry 0.6 g (3 w % with respect to the solid feed material) of a magnetite powder ( $Fe_3O_4$ , particle size:  $\times 50=1-3 \mu m$ ,  $\times 90=4-10 \mu m$ ) coated with 1.35 w % of a solid methyl silicone resin (melting range 35-55° C.) from a toluene solution according to WO 2015/110555 dispersed in 3.6 g of an 0.1 w % aqueous solution of a non-ionic surfactant (general formula  $RO(CH_2CH_2O)_xH$ ,  $x=8$ , derived from a  $C_{10}$  Guerbet alcohol  $ROH$ , wherein  $R=C_{10}H_{21}$ ) was added (step 3). This slurry was stirred for 15 min with a 30 mm pitch blade stirrer at 1400 rpm corresponding to an energy input of approx. 0.7 kWh/m<sup>3</sup> (step 3a).

The resulting dispersion is pumped with a rate of 6 l/h to an Eriez L4 WHIMS lab-scale magnetic separator equipped with a 4x2 mm wedged wire matrix at a magnetic field strength of 0.7 T (step 4). After completion of the feed addition the matrix is flushed with water (step 4a). The combined dispersion and flush water are collected as tailings. Afterwards the magnetic field was switched off and the magnetic fraction containing the magnetite molybdenite agglomerates are flushed out from the matrix and collected separately yielding the magnetic concentrate. The elemental composition of both fractions was analyzed.

|             | non-magnetic fraction | magnetic fraction |
|-------------|-----------------------|-------------------|
| dry mass    | 8.28 g                | 11.65 g           |
| Cu-content  | 1.58%                 | 1.10%             |
| Mo-content  | 5.08%                 | 48.27%            |
| Cu-recovery | 50.2%                 | 49.8%             |
| Mo-recovery | 7.0%                  | 93.0%             |

### Example 2: Enriched Mo-Ore

The experimental conditions were as in example 1 except that 100 mg (0.5%) of the liquid mixed hydrocarbon was used.

|             | non-magnetic fraction | magnetic fraction |
|-------------|-----------------------|-------------------|
| dry mass    | 15.73 g               | 3.88 g            |
| Cu-content  | 1.24%                 | 1.68%             |
| Mo-content  | 30.51%                | 39.68%            |
| Cu-recovery | 75.0%                 | 25.0%             |
| Mo-recovery | 75.7%                 | 24.3%             |

### Example 3: Enriched Mo-Ore

The experimental conditions were as in example 1 except that 200 mg (1.0%) of the liquid mixed hydrocarbon was used.

|             | non-magnetic fraction | magnetic fraction |
|-------------|-----------------------|-------------------|
| dry mass    | 14.94 g               | 4.89 g            |
| Cu-content  | 1.32%                 | 1.38%             |
| Mo-content  | 27.75%                | 42.19%            |
| Cu-recovery | 74.5%                 | 25.5%             |
| Mo-recovery | 66.8%                 | 33.2%             |

### Example 4: Enriched Mo-Ore

The experimental conditions were as in example 1 except that 300 mg (1.5%) of the liquid mixed hydrocarbon was used.

|             | non-magnetic fraction | magnetic fraction |
|-------------|-----------------------|-------------------|
| dry mass    | 11.63 g               | 8.08 g            |
| Cu-content  | 1.49%                 | 1.12%             |
| Mo-content  | 18.68%                | 49.69%            |
| Cu-recovery | 65.7%                 | 34.3%             |
| Mo-recovery | 35.1%                 | 64.9%             |

## Comparative Example 1: Enriched Mo-Ore

The experimental conditions were as in example 1 except that 80 mg (0.4%) of the liquid mixed hydrocarbon was used.

|             | non-magnetic fraction | magnetic fraction |
|-------------|-----------------------|-------------------|
| dry mass    | 16.14 g               | 3.66 g            |
| Cu-content  | 1.26%                 | 1.73%             |
| Mo-content  | 29.85%                | 39.35%            |
| Cu-recovery | 76.2%                 | 23.8%             |
| Mo-recovery | 77.0%                 | 23.0%             |

## Comparative Example 2: Enriched Mo-Ore

The experimental conditions were as in example 1 except that 60 mg (0.3%) of the liquid mixed hydrocarbon was used.

|             | non-magnetic fraction | magnetic fraction |
|-------------|-----------------------|-------------------|
| dry mass    | 16.88 g               | 2.65 g            |
| Cu-content  | 1.29%                 | 1.76%             |
| Mo-content  | 26.22%                | 40.38%            |
| Cu-recovery | 82.4%                 | 17.6%             |
| Mo-recovery | 82.2%                 | 17.8%             |

Comparing examples 1 to 4 and comparative examples 1 and 2 show that in the case of the given Mo feed material the amount of added hydrocarbon strongly determines the Mo recovery in the inventive separation process and that with amounts of hydrocarbons above the one described in the art the separation process becomes more efficient.

## Example 5: Enriched Mo-Ore

In a buffled beaker 20 g (19.3 g dry mass) of an enriched solid Mo-ore, containing 35.5% Mo as Molybdenite ( $\text{MoS}_2$ ) and 1.6% Cu mainly as Chalcopyrite ( $\text{CuFeS}_2$ ), are provided. The material has a particle size d80 of 40  $\mu\text{m}$ . The material was dispersed in 60 g of filtrated river water yielding a solid content of 25 w % (step 1). This dispersion was stirred with an Ultra Turrax T25 stirrer for 5 min at 10000 rpm (step 1 b).

To this dispersion 1.0 g corresponding to a concentration of 50000 g/t solid of the same liquid mixed hydrocarbon as used in example 1 (boiling range of 149-213° C., dynamic viscosity of  $1.2 \cdot 10^{-6} \text{ m}^2/\text{sec}$  (20° C.)) (step 2) and a slurry 0.6 g (3 w % with respect to the solid feed material) of a magnetite powder (the same as used in example 1) coated with 1.35 w % of a solid methyl silicone resin (melting range 35-55° C., the same as used in example 1) from a toluene solution according to WO 2015/110555 dispersed in 4 g isopropanol was added (step 3) were added thus, omitting the stirring step 2a.

This slurry was stirred for 15 min with a 30 mm pitch blade stirrer at 1400 rpm corresponding to an energy input of approx. 0.7 kWh/m<sup>3</sup> at a specific power input of 3 kW/m<sup>3</sup> (step 3a). The resulting dispersion is pumped with a rate of 5 6 l/h to an Eriez L4 WHIMS lab-scale magnetic separator equipped with a 4x2 mm wedged wire matrix at a magnetic field strength of 0.7 T (step 4). After completion of the feed addition the matrix is flushed with water (step 4a).

The combined dispersion and flush water are collected as 10 tailings. Afterwards the magnetic field was switched off and the magnetic fraction containing the magnetite molybdenite agglomerates are flushed out from the matrix and collected 15 separately yielding the magnetic concentrate. The elemental composition of both fractions was analyzed.

|             | non-magnetic fraction | magnetic fraction |
|-------------|-----------------------|-------------------|
| dry mass    | 7.55 g                | 12.37 g           |
| Cu-content  | 2.54%                 | 1.49%             |
| Mo-content  | 23.07%                | 46.09%            |
| Cu-recovery | 50.9%                 | 49.1%             |
| Mo-recovery | 23.4%                 | 76.6%             |

## Example 6: Enriched Mo-Ore

The experimental conditions were as in example 7 except that the stirring of the water and the liquid mixed hydrocarbon with the Ultra Turrax stirrer in step 1b was omitted.

Instead, after the addition of the liquid mixed hydrocarbon and before the addition of the magnetite carrier the mixture is vigorously stirred with an Ultra Turrax T25 for 5 min at 10000 rpm (spec. energy input approx. 300 kWh/m<sup>3</sup> 35 at a spec. power of 3600 kW/m<sup>3</sup>) (Step 2a).

|             | non-magnetic fraction | magnetic fraction |
|-------------|-----------------------|-------------------|
| dry mass    | 5.60 g                | 14.31 g           |
| Cu-content  | 4.08%                 | 1.13%             |
| Mo-content  | 3.69%                 | 51.03%            |
| Cu-recovery | 58.5%                 | 41.5%             |
| Mo-recovery | 2.8%                  | 97.2%             |

## Example 7: Enriched Mo-Ore

In a buffled beaker 122.8 g of an enriched solid Mo-ore (120.0 g dry mass), containing 30.0% Mo as Molybdenite ( $\text{MoS}_2$ ) and 1.5% Cu mainly as Chalcopyrite ( $\text{CuFeS}_2$ ), are provided. The material has a particle size d80 of 30  $\mu\text{m}$ . The material was dispersed in 357 g of filtrated river water yielding a solid content of 25 w % (step 1) and mixed with an Ultra Turrax T50 stirrer for 5 min at 6000 rpm (spec. energy input approx. 150 kWh/m<sup>3</sup>). To this dispersion 3000 mg of the same liquid mixed hydrocarbon as used in example 1 (boiling range of 149-213° C., dynamic viscosity of  $1.2 \cdot 10^{-6} \text{ m}^2/\text{sec}$  (20° C.)) (step 2), corresponding to a concentration of the hydrocarbon of 25000 g/t solid, were added (step 2). 55 Afterwards this dispersion was vigorously mixed with an Ultra Turrax T50 stirrer for additional 2 min at 6000 rpm (spec. energy input approx. 50 kWh/m<sup>3</sup>) (Step 2a).

Subsequently to this slurry 3.6 g (3 w % with respect to 60 the solid feed material) of magnetite powder (the same as in example 1) coated with 1.35 w % of the same solid methyl silicone resin as used in example 1 from a toluene solution according to WO 2015/110555 dispersed in 21.6 g of an 0.1

w % aqueous solution of the same non-ionic surfactant as used in example 1 was added (step 3).

This slurry was stirred for 15 min with a 45 mm pitch blade stirrer at 1000 rpm corresponding to an energy input of approx. 0.5 kWh/m<sup>3</sup> (step 3a). The resulting dispersion is pumped with a rate of 6 l/h to an Eriez L4 WHIMS lab-scale magnetic separator equipped with a 4x2 mm wedged wire matrix at a magnetic field strength of 0.7 T (step 4). After completion of the feed addition the matrix is flushed with water (step 4a). The combined dispersion and flush water are collected as tailings which are filtered and dried. Afterwards the magnetic field was switched off and the magnetic fraction containing the magnetite molybdenite agglomerates are flushed out from the matrix and collected separately yielding the magnetic concentrate.

|             | non-magnetic fraction | magnetic fraction |
|-------------|-----------------------|-------------------|
| dry mass    | 48.75 g               | 74.80 g           |
| Cu-content  | 1.93%                 | 0.99%             |
| Mo-content  | 5.76%                 | 47.78%            |
| Cu-recovery | 56.1%                 | 43.9%             |
| Mo-recovery | 7.3%                  | 92.7%             |

The magnetic fraction of the magnetic separation of step 4 was filtered to obtain 84.15 g of wet filter cake with a water content of 11.1% and samples were taken for the corresponding elemental analyses. The elemental composition of both fractions was analyzed. For the recovery of the magnetite the remaining 16.88 g of the filtrated but not dried solid magnetic fraction (corresponds to 15.00 g dry mass) were suspended in a solution of 500 g of filtered river water and 1.35 g of the same non-ionic surfactant as used in step 3 (steps 5 and 5a) and stirred with a 72 mm pitch blade stirrer for 10 min at 300 rpm (corresponding to an energy input of approx. 0.04 kWh/m<sup>3</sup>) (step 5b).

Afterwards the resulting slurry is pumped to a lab-scale MIMS magnetic separator device as described in WO 2014/068142 (step 6) with a feed flow of 24.4 l/h a flush water flow of 12 l/h for the resulting magnetic fraction and a flow of 7.4 l/h for the magnetic fraction and a resulting flow of 29 l/h flow of the non-magnetic fraction. The resulting magnetic fraction which contained mainly the magnetite carrier material and the non-magnetic fraction containing the concentrated mineral target particles were filtered and their elemental composition was analyzed.

|             | non-magnetic fraction | magnetic fraction |
|-------------|-----------------------|-------------------|
| dry mass    | 0.71 g                | 14.30 g           |
| Cu-content  | 0.24%                 | 0.99%             |
| Mo-content  | 4.23%                 | 48.94%            |
| Cu-recovery | 1.2%                  | 98.8%             |
| Mo-recovery | 0.4%                  | 99.6%             |

The invention claimed is:

1. A process for separating at least one first material from a mixture comprising this at least one first material, at least one second material and at least one third material, which comprises at least the following steps:

(A) providing a mixture comprising at least one first material, at least one second material, at least one third

material and at least one hydrocarbon in an amount of 0.5% by weight or more, based on the sum of mixture, in the presence or absence of at least one dispersion medium,

- 5 (B) optionally, adding at least one dispersion medium to the mixture obtained in step (A) in order to obtain a dispersion,  
10 (C) treating the dispersion from step (A) or (B) with at least one hydrophobic magnetic particle, so that the at least one first material and the at least one magnetic particle agglomerate,  
15 (D) separating the adduct from step (C) from the mixture by application of a magnetic field,  
(E) optionally, dissociation of the adduct which has been separated off in step (D) in order to obtain the at least one first material and the at least one magnetic particle separately.

2. The process according to claim 1, wherein the at least one first material and the at least one second material are 20 hydrophobic metal compounds and the at least one third material is a hydrophilic metal compound.

25 3. The process according to claim 1, wherein the at least one hydrocarbon is selected from the group consisting of crude oil derivatives, mineral oils, mineral waxes, vegetable oils, biodiesel, diesel and mixtures thereof.

4. The process according to claim 1, wherein the at least one hydrocarbon has a flash point of at least 20° C.

5. The process according to claim 1, wherein the at least one first material is a sulfidic molybdenum ore and the at least one second material is a sulfidic copper ore.

30 6. The process according to claim 1, wherein the at least one third material is selected from the group consisting of oxidic and hydroxidic metal compounds.

35 7. The process according to claim 1, wherein the at least one magnetic particle is selected from the group consisting of magnetic metals and mixtures thereof, ferromagnetic alloys of magnetic metals and mixtures thereof, magnetic iron oxides, cubic ferrites of the general formula (III)



40 where

M is selected from among Co, Ni, Mn, Zn and mixtures thereof and

x is  $\leq 1$ ,

hexagonal ferrites and mixtures thereof.

45 8. The process according to claim 1, wherein the dispersion medium in step (A) is water.

9. The process according to claim 1, wherein the mixture comprising at least one first material, at least one second material and at least one third material is milled to particles having a size of from 100 nm to 100  $\mu$ m before or during step (A).

50 10. The process according to claim 1, wherein the mixture of step (A) or, if step (B) is carried out, the dispersion obtained from step (B) is mixed vigorously such that energy in an amount of 150 kWh/m<sup>3</sup> or more is introduced into the mixture prior to step (C).

55 11. The process according to claim 1, wherein a hydrophobizing agent is added in step (A).

60 12. The process according to claim 1, wherein at least one hydrocarbon in an amount of 1% by weight or greater.

\* \* \* \* \*